

# UNITED STATES PATENT OFFICE.

JOSEPH E. JOHNSON, JR., OF NEW YORK, N. Y.; MARGARET HILLES JOHNSON EXECUTRIX OF SAID JOSEPH E. JOHNSON, JR., DECEASED.

## PRODUCTION OF FERROMANGANESE.

1,354,490.

Specification of Letters Patent.

Patented Oct. 5, 1920.

No. Drawing.

Application filed July 23, 1918. Serial No. 246,345.

To all whom it may concern:

Be it known that I, JOSEPH E. JOHNSON, Jr., a citizen of the United States, residing at New York, in the county of New York, 5 State of New York, have invented certain new and useful Improvements in Production of Ferromanganese; and I do hereby declare the following to be a full, clear, and exact description of the invention, such 10 as will enable others skilled in the art to which it appertains to make and use the same.

Ferro-manganese alloys are used in large quantities in the manufacture of steel. It 15 is desirable to have them high in manganese and low in carbon for two reasons, to wit:

First, the lower the percentage of manganese in the ferro-manganese alloy, the more troublesome and expensive is its employment 20 as an addition in the manufacture of steel; for the reason that as the percentage of manganese in the ferro-manganese alloy declines, the total amount of the other constituents of the alloy increases, thereby introducing into the steel a correspondingly 25 increased proportion of these other constituents of the alloy, with proportionate disadvantage.

Secondly, it is found that the presence 30 of a relatively large amount of carbon, in proportion to the manganese, in ferro-manganese alloys containing both iron and carbon, lowers the availability of such alloys in the manufacture of steel for many uses.

35 For instance, in order to introduce into a bath of molten iron or steel a sufficient quantity of manganese, it is, in many cases, not feasible to employ, for that purpose, spiegeleisen, even though the spiegeleisen 40 may have as high as 20% of manganese; for the reason that spiegeleisen having that content of manganese contains about 5% of carbon, so that to add to the steel a sufficient amount of spiegeleisen to give the steel the 45 desired manganese content would involve, in many cases, the simultaneous introduction of an amount of carbon beyond the permissible limit. On the other hand, the carbon content of a manganese alloy containing

50 both iron and carbon rises but slowly with increasing proportions of manganese in the alloy, so that a ferro-manganese alloy containing as high as 80% of manganese contains only 6 to 6½% of carbon, for which 55 reason, by the use of such an alloy, the op-

erator is enabled to give to the steel the desired manganese content while restricting the amount of carbon simultaneously introduced to a feasible and acceptable minimum.

For the foregoing reasons, standard ferro-manganese containing 80% of manganese had, for most uses, previous to the scarcity of manganese brought about by the present war, driven out commercially the use of low manganese alloys, even in the manufacture 60 of high carbon steels.

The high grade manganese ores required, in accordance with the methods practised in the art at the present time, to make the standard ferro-manganese alloy containing 70 80% of manganese occur in the United States in very limited amounts, whereas low grade manganese ores (that is to say, ores low in manganese) occur in much greater quantities.

75 Ferro-manganese alloys may be produced either in the electric furnace or in the iron blast furnace. Both of these methods, as at present practised, are open to serious objection. For instance, in the electric furnace, 80 the consumption of power is high, running from 6,000 to 10,000 kilowatt hours per ton of manganese. The cost of this power, in many localities, exceeds, at present, the normal selling price obtained for the manganese 85 alloy in times of peace, so that the production of ferro-manganese alloys in the electric furnace is, under present conditions, only feasible if an extremely high price can be obtained for the product, or where by 90 reason of peculiarly favorable local conditions, low cost electric power is available.

On the other hand, the production of ferro-manganese alloys in the ordinary iron blast furnace is accompanied with very 95 considerable losses of manganese, due to the fact first, that the manganese has a greater affinity for silica and unites with it to form silicate of manganese, which passes out into slag, and secondly, that the manganese is volatilized in very considerable amounts and passes out of the top of the furnace as a fume, which has been found to be practically irrecoverable.

100 In the electric furnace, it is possible to 105 greatly reduce the slagging loss and at the same time to have a relatively small loss from fume, by maintaining the hearth temperature of the furnace sufficiently high. So also, the slagging loss of manganese may 110

be reduced by increasing the heat in the smelting zone or hearth of the existing blast furnace, but this cannot be done in ordinary blast furnace practice without materially increasing the heat in the furnace shaft, and this increase in heat in the furnace shaft (where the normal temperature is, in any event, unduly high) is found to increase the volatilization loss; so that, in the best blast furnace practice, the loss in manganese runs from 15 to 25%.

My investigations of the iron blast furnace have shown that the great difficulty with the process as at present practised is the relatively small amount of high temperature heat which can be produced for the hearth in comparison with the amount of low temperature heat simultaneously produced and which is only useful in the shaft.

In the case of the iron blast furnace, this is compensated to a considerable extent by the fact that iron ore is reducible to a very large extent by the carbon monoxid gas generated in the hearth, and therefore, a large percentage of the total work of the iron blast furnace is done in the shaft by the reducing action of the carbon monoxid gas rising through it.

Different conditions, however, prevail in the reduction of manganese in manganese blast furnace practice. Carbon monoxid reduces manganese oxid to a much smaller extent than it does iron oxid, and, therefore, a much smaller portion of the total work of reduction takes place in the shaft, the far larger proportion of the reduction being effected in the hearth and by the direct action of carbon instead of by the action of carbon monoxid. Consequently, the requirements of heat in the hearth of the manganese blast furnace are greatly increased, whereas the requirements of heat in the shaft of the manganese blast furnace are relatively small. Consequently, blast furnaces for the production of ferro-manganese use about three times the amount of fuel per ton of metal that is used in blast furnaces for the production of iron, although the amount of heat required for reduction is but slightly greater than in the case of iron. This results in an enormous excess of heat in the shaft of the manganese blast furnace, as above indicated, and this excess of heat is accompanied by a tremendous volume of gas, both of which conditions tend greatly to promote the volatilization of the manganese.

Furthermore, the conditions of high temperature, greater gas volume, and the presence of large quantities of manganese oxid fume have a violent destructive effect on the lining of the furnace, so that the life of the lining of a blast furnace for the production of ferro-manganese is but a fraction 65 of the life of the same furnace when pro-

ducing pig iron. So also, in ferro-manganese blast furnace practice, the large quantity of fuel which reaches the hearth gives a corresponding amount of silica in the form of coke ash, and this takes a corresponding toll of manganese in the form of manganese silicate passing out in the slag.

The output in metal of a given blast furnace depends primarily upon the amount of fuel that it can burn in the hearth, and any cause which leads to an increased consumption of fuel per ton of metal, reduces the metal output by a more than proportional amount. Consequently, inasmuch as the fuel consumption in ferro-manganese blast furnace practice is about three times as high as the fuel consumption in pig iron production, the metal output of ferro-manganese blast furnaces is only about one-third or less than that of the same furnaces when used in the production in pig iron. This low output, together with the short life of the furnace lining, and the high cost for re-lining, increases very considerably the cost of making ferro-manganese, over that of making pig iron, entirely apart from the cost of ferro-manganese ore.

A further consideration of importance is that lean ores require more fuel for their smelting than richer ones, so that as the ores of manganese become leaner, the fuel requirements rise still further, which adds to all of the unfavorable conditions hereinbefore described.

I have found that the difficulties described as existing in the production of ferro-manganese in the blast furnace can be enormously diminished by a procedure which essentially and radically changes the heat conditions prevailing in the furnace, and particularly by a procedure which permits the operator to proportion the amount of shaft heat and of hearth heat to one another according to their respective requirements.

Thus, I have ascertained that if the nitrogen introduced as a constituent of the air in the ordinary ferro-manganese blast furnace practice is substantially diminished, or greatly reduced, so that the blast employed is rich in oxygen, it is possible to so radically alter the furnace conditions as to practically revolutionize the mode of operation of the furnace and the results obtained.

In the practice of the invention, I lower the relative amount of nitrogen and increase the relative amount of oxygen in the blast until I obtain an adjustment of the composition appropriate to the proportionate amount of hearth heat and of shaft heat desired. The elimination of the nitrogen has the cumulative effect of increasing the amount of high temperature heat obtainable per unit of fuel and of reducing to an enormous extent the amount of gas which by its physical heat-carrying capacity serves

to carry the heat out of the stack, where it is necessary and desirable, up into the hearth where, beyond a moderate amount, it is not only unnecessary, but harmful. Furthermore, the result of the increased heat per pound of fuel is to reduce the fuel required per pound of metal smelted, and this, in turn, makes a still further proportionate reduction of the amount of gas per pound of metal passing out of the hearth.

In practice, I find that, by the practice of the invention, I am able to reduce the amount of fuel to less than half of that now required in ferro-manganese blast furnace practice. So also, I very considerably reduce the manganese loss for the reason, first, that the reduction of the silica in the charge, due to the reduction of it in the coke, combined with the increased temperature in the hearth lessens the manganese loss in the slag so as to bring it down to a small percentage of its present proportions, and, secondly, because the enormous reduction in the amount and temperature of the gas in the shaft of the furnace cuts down the loss of manganese by volatilization to a highly important extent.

Furthermore, the practice of the invention permits an important reduction in the expense for lining, maintenance, etc., for the reason that the reduced volume and temperature of the gases and the reduction of their content of manganese fume decreases the wear on the lining of the furnace to a fraction of its present amount. Furthermore, because of the much smaller amount of fuel required and the smaller proportionate amount of gas evolved per pound of fuel, it is feasible to reduce the size of the furnace required for a given output, to a fraction of the present size. The increased life of the lining, and the smaller size of the furnace required reduces the expense for refractories and for maintenance and overhead, to a fraction of their present amounts.

In addition to the hereinbefore described advantages of the invention, it permits me to introduce certain other features not commercially practicable in the ordinary ferro-manganese blast furnace practice. Thus, with the increased hearth heat available, I can reduce a considerable percentage of silicon and cause it to unite with the ferro-manganese with the result of forcing down the carbon contents of the alloy.

I can, if so desired, add a further step to the process, by subjecting the alloy, while still in the liquid condition, but after it has been tapped off into a separate vessel, to the action of oxid of iron or oxid of manganese, or both, with the result that these oxids attack the silicon of the alloy and reduce it to silica, which, uniting with a portion of the oxid unreduced, passes off as slag, the metal reduced from the oxid entering the

alloy. By this means I can produce an alloy high in manganese and low in both carbon and silicon.

Moreover, on account of the greatly reduced losses, I am able to make ferro-manganese of higher grade from a given ore than can be done in the ordinary ferro-manganese blast furnace practice; or I can use the relatively low grade manganese ores for the production of standard 80% ferro-manganese in the production of that alloy, thereby further decreasing the cost of the alloy and making available for its production many ores which are excluded in the present practice.

What I claim is:

1. The method of producing in a blast furnace, alloys of iron, high in manganese, which comprises blowing the furnace charge (containing carbon, iron and manganese) with a blast richer in oxygen and poorer in nitrogen than the atmosphere, the relative oxygen and nitrogen content of the blast being so proportioned that an increase in hearth temperature is produced sufficient to obtain the desired high manganese content in the alloy, with accompanying decrease in the amount and temperature of the gases traversing the shaft of the furnace, whereby manganese losses are diminished, and a saving of fuel per unit of alloy output is effected; substantially as described.

2. The method of producing in a blast furnace, alloys of iron, high in manganese, and low in silicon and carbon, which comprises blowing the furnace charge (containing carbon, iron, manganese and silicon) with a blast richer in oxygen and poorer in nitrogen than the atmosphere, the relative oxygen and nitrogen content of the blast being so proportioned that an increase in hearth temperature is produced sufficient to obtain the desired high manganese content in the alloy and to likewise increase the content of silicon at the expense of the carbon content of the alloy and with accompanying decrease in the amount and temperature of the gases traversing the shaft of the furnace, and then treating the resultant alloy product while still in a liquid condition with a silicon-oxidizing slag, thereby lowering the proportion of silicon in the final alloy product; substantially as described.

3. The method of producing in a blast furnace, alloys of iron, high in manganese and low in silicon and carbon, which comprises blowing the furnace charge (containing carbon, iron, manganese and silicon) with a blast richer in oxygen and poorer in nitrogen than the atmosphere, the relative oxygen and nitrogen content of the blast being so proportioned that an increase in hearth temperature is produced sufficient to obtain the desired high manganese content in the alloy and to likewise increase the con-

- tent of silicon at the expense of the carbon content of the alloy and with accompanying decrease in the amount and temperature of the gases traversing the shaft of the furnace, and then treating the resultant alloy product while still in a liquid condition with a silicon-oxidizing slag comprising at least one of the oxids of the constituent metals of the alloy other than silicon, thereby lowering the proportion of silicon in the final alloy product and introducing therein an additional proportion of the metal of the reduced oxid; substantially as described.
4. The method of producing in a blast furnace, alloys of iron, high in manganese, and low in silicon and carbon, which comprises blowing the furnace charge (containing carbon, iron, manganese and silicon) with a blast richer in oxygen and poorer in

nitrogen than the atmosphere, the relative 20 oxygen and nitrogen content of the blast being so proportioned that an increase in hearth temperature is produced sufficient to obtain the desired high manganese content in the alloy and to likewise increase the content of silicon at the expense of the carbon content of the alloy and with accompanying decrease in the amount and temperature of the gases traversing the shaft of the furnace, and then treating the resultant alloy 25 product while still in a liquid condition with a silicon-oxidizing slag, comprising oxid of manganese, thereby lowering the proportion of silicon in the final alloy product and raising the proportion of manganese 30 therein; substantially as described.

In testimony whereof I affix my signature.  
JOSEPH E. JOHNSON, JR.